

## UNITED STATES PATENT OFFICE

2,689,163

TANNING AGENT AND METHOD OF MAKING  
AND USING SAME

Maxime Paquet, Pougues-les-Eaux, France

No Drawing. Application April 17, 1951,  
Serial No. 221,519Claims priority, application France  
October 27, 1948

26 Claims. (Cl. 8—94.25)

1

The present invention relates to a novel tanning product, the method of manufacturing said product, a tanning bath in the preparation of which this novel tanning product is employed and a process of tanning therewith.

The present invention is a continuation-in-part of my copending application filed October 18, 1949 having the Serial No. 122,125.

The use of soluble zirconium compounds as tanning agents is known in the prior art. More particularly, solutions containing soluble zirconium sulfate or chloride salts have been utilized in tanning baths but, non-uniform and incomplete tanning results have been obtained. The prior art has attempted to remedy these defects by adding a soluble sulfate compound to the tanning bath containing the zirconium compound to improve the extent of tanning. It has also been suggested to add water soluble silicic acid compounds or water soluble silicates to the zirconium containing tanning liquor in order to obtain improved coloration of the hide or skin. However, thorough tanning to give uniform results as to color, feel and appearance have not been obtained when utilizing a soluble zirconium compound in accordance with prior art methods.

It has now been discovered that excellent tanning results are obtainable by using tanning liquors in the preparation of which is employed a soluble zirconium salt absorbed in a silica gel. This tanning agent is preferably produced directly by reaction from a sodium silico-zirconate with a concentrated mineral acid at elevated temperatures, whereby a complex water soluble zirconium salt is formed simultaneous with, and imbedded in the pores of, the silica gel. This resultant product, which is in the form of a pulverulent solid, can be used directly in the tanning bath by the slow dissolution of the complex zirconium salt out of the pores of the insoluble silica gel, to function as the tanning agent for the animal skins in the presence of the silica gel. Thus, the tanning bath is prepared by dissolving the tanning agent, namely the zirconium salt absorbed by the silica gel, in water. This tanning agent will slowly dissolve so that the bath actually contains not only zirconium salts absorbed by silica gel, but also the liberated zirconium salt in direct solution in the water forming the base of the bath. This liberation of the zirconium salt occurs over an extended period of time at a substantially uniform rate.

As the tanning is carried out during the extended period of the dissolving process, there will be available for the tanning action, during at least the greater part of such period, a substan-

tially uniform concentration of liberated zirconium salt ensuring uniform tanning action. In this relationship, the silica gel acts as a surface active agent (not as a tanning agent) to assist the zirconium salt in its affinity for and penetration into the fibers of the skin. The leather obtained by the instant process is very white, very full, has an excellent "hand" or feel, and a very beautiful appearance.

Accordingly, an object of the instant invention is to provide a novel and superior tanning agent, comprising a complex zirconium salt absorbed in the pores of a silica gel.

Another object of the present invention is the development of a process of directly producing this novel tanning agent from sodium silico-zirconate.

A further object of this invention is the use of these novel tanning agents in the preparation of a tanning bath to produce a superior quality leather.

A further object of this invention is the development of a process of tanning with a complex soluble zirconium salt embedded in a silica gel.

Further objects and advantages of the present invention will be apparent from the following description.

As a result of my discovery, the disadvantages of tanning with a zirconium salt are eliminated and a superior leather obtained by using a silica gel as the absorbent carrier for a complex soluble zirconium salt. This silica gel remains insoluble in the tanning bath, exerting no tanning action on the hides or skins. However, the surface active property of the gel functions to alter the rate of dissolution and thereby also the tanning action of the zirconium salts so as to produce a thorough and complete tanning. While the invention is not limited to any particular theory, it is apparent that the action of the silica gel is essentially physico-chemical in nature. By virtue of the greater affinity of the zirconium salt for the fibers of the skin and due to the regulated and slow tanning action, a uniform tanning with a high utilization of the tanning agent is effected, rendering the instant process commercially desirable.

The quantity of silica gel utilized to obtain the superior results of the instant invention based on the amount of soluble zirconium salt is about 0.1 mol.—2 mol. of silica gel for each mole of  $ZrO_2$ , the preferred range being about 0.2—1.3 mol  $SiO_2$  for 1 mol  $ZrO_2$ . The appearance and "hand" of the leather depends on the  $SiO_2/ZrO_2$  ratio.

The soluble zirconium salts utilized are sulfates,

chlorides, nitrates or the like. The molecular composition for the sulfate salt is represented by the following ratio, 1 mol.  $ZrO_2$  for 0.8-2.2 mol.  $SO_3$ , the preferred range being 1 mol.  $ZrO_2$ :1.2-1.8 mol.  $SO_3$ . The molecular ratio for the chloride salt is 1 mol.  $ZrO_2$ :1.6-4 mol. HCl, preferably 1 mol.  $ZrO_2$ :1.8-2.6 mol. HCl.

Another embodiment of the instant invention is the development of a process for producing the complex soluble zirconium salt dispersed in a silica gel directly and simply from a sodium silico-zirconate by treatment with a concentrated mineral acid at temperatures above 105° C. The sodium silico-zirconate can be economically produced from the mineral zircon, a zirconium silicate, by calcination in the presence of sodium carbonate. More specifically, the transformation of zircon into the sodium silico-zirconate (e. g.  $Na_2SiZrO_5$ ) can be carried out by fritting the powdered zircon with an excess of about 5% sodium carbonate at about 1000° C. for two hours. The fritted mass containing the sodium silico-zirconate, is subsequently treated with a concentrated acid, preferably sulphuric, hydrochloric, nitric acid or non-precipitating mixtures thereof, the concentration of the acid being sufficient to raise the temperature of this exothermic reaction above 105° C. and preferably to 110°-120° C. The exothermicity of this reaction vaporizes the water, resulting thereby in a substantially dry end product. The amount of acid utilized must be sufficient to transform all of the  $Na_2O$  and all of the acid soluble  $ZrO_2$  into the water soluble salts of the specific mineral acid used. Illustratively, using  $H_2SO_4$ , the  $ZrO_2$  and  $Na_2O$  combine with the  $H_2SO_4$  to form a complex salt of  $Na_2SO_4$  and zirconium sulfate, having the molecular composition represented by the  $ZrO_2:SO_3$  ratio specifically set forth above.

The concentration of the acid must be such that an exothermic reaction ensues. When using sulfuric acid the concentration in relation to the water in the mass is 35°-60° Bé. which is equivalent to a specific gravity of 1.32 to 1.71 or a concentration of 41-78% by weight. A more concentrated acid, such as represented by 66° Bé. (93%  $H_2SO_4$ ), is added to a paste of sodium silico-zirconate already containing water, so that a final concentration of 35-60° Bé.  $H_2SO_4$  is obtained. By regulating the concentration of the acid within the above specified limits, the character of the gel and of the zirconium salt can be varied so as to render them especially suitable for obtaining varied tanning results. By maintaining the amount of acid constant, and decreasing the amount of water added to the sodium silico-zirconate to form the paste, the concentration of the acid is increased and the temperature of the reaction is elevated resulting in an enlargement of the grains of silica gel and a decrease in the absorptive capacity of the gel, and in a smaller amount of combined water with the complex zirconium salt which is characterized by a slower dissolution of the zirconium salt in water. When maintaining the amount of the acid constant and increasing the amount of water added to the sodium silico-zirconate to form the paste, the concentration of the acid is decreased and the temperature is lowered, resulting in a more voluminous and absorptive silica gel composed of smaller grains, and in a greater amount of combined water with the complex salt of zirconium. Consequently, variations in the temperature of the reactions, in the concentrations of the acids, and in the  $ZrO_2:SO_3$  ratio modify the tanning

properties of the resultant product which is a pulverulent solid of a complex salt of zirconium embedded and absorbed in a silica gel.

Hydrochloric acid may also be utilized to attack the sodium silico-zirconate, but in concentrations represented by 13°-22° Bé., preferably 16°-20° Bé., the broad range being equivalent to a specific gravity of 1.10-1.18 or 20-36% HCl by weight, in amounts necessary to convert the total  $Na_2O$  content to  $NaCl$  and the  $ZrO_2$  content into a soluble zirconium chloride salt having the molecular composition previously discussed. Similarly to the use of sulfuric acid, the concentration and quantity of HCl can be varied within the above specified limits, taking into consideration the sodium silico-zirconate to be treated and the results desired. Thus, the speed of dissolution of the zirconium compound in the tanning solution, and the physical characteristics of the silica gel as to grain size and absorptive properties, can be regulated by adjusting the concentration of the acid, the temperature of the acid attack and the cooling of the reaction mass.

Nitric acid can also be used to attack the sodium silico-zirconate. However, the difference in the molecular weights of the mineral acids require different amounts and concentrations thereof to produce the desired tanning product. Accordingly, the concentration of the nitric acid lies within the range of 20° Bé. and 40° Bé., which is equivalent to a specific gravity of 1.16 to 1.38 or a weight percentage of 26 to 63%  $HNO_3$ .

The desired concentrations of the acids are those which are present in the acid solutions at the time of bringing it into contact with the pulverized frit of sodium silico-zirconate. These concentrations can be obtained by either mixing the necessary amount of water with the commercial acid, or preferably by making a paste of the fritted mass with water to which a strong acid is subsequently added. In lieu of single acids, non-precipitating mixed acids such as non-precipitating mixtures of sulphuric and nitric acids, etc., may be utilized, the degree of dilution of the acids being dependent on the molecular weight of the acids used.

This economical process of producing the zirconium tanning agent in the form of a pulverulent solid which can be used directly in the tanning bath has rendered this tanning process commercially feasible. To date, in spite of the advantages of zirconium tanning, the high cost of the zirconium salts has prohibited its use on an industrial scale. However, the zirconium minerals are inexpensive, zircon being one of the cheapest. According to the instant process of producing the tanning agent directly from the mineral, zirconium tanning is rendered economical as well as productive of a superior leather. Although zircon is the preferred mineral, other zirconium minerals such as zirkites, baddeleyites, etc., can be utilized alone or admixed with silica or zircon. Furthermore, the instant process produces good yields of tanning agents possessing a high degree of purity.

The following examples are additionally illustrative of the process of obtaining the zirconium tanning agent of the instant invention, and are not to be construed as limiting the scope thereof.

#### EXAMPLE A

250 kgs. of silico-zirconate of sodium (containing substantially 245 kgs. of  $ZrO_2SiO_2Na_2O$  and 5 kgs. of impurities), preferably ground to a powder corresponding to 100 mesh, are trans-

formed into a paste by adding 210 liters of water. Then 220 kgs. of sulfuric acid at 66° Bé. (i. e. 93% of pure  $H_2SO_4$ ) are rapidly added to the paste with vigorous stirring.

The reaction is exothermic and the temperature increases rapidly to above 110° C. and a part of the added water is vaporized thereby. Substantially all of the silica is transformed into a voluminous gel having a great absorbing capacity which is in the form of coarse grains substantially completely insoluble in water.

The  $ZrO_2$  and the  $Na_2O$  combine with the  $H_2SO_4$  in the form of a complex salt which is soluble in water and is absorbed by the silica gel.

600 kgs. of tanning product are thereby obtained, having approximately the following analysis:

|                                                                                                         | Percent     |
|---------------------------------------------------------------------------------------------------------|-------------|
| Soluble $ZrO_2$ -----                                                                                   | about 20    |
| Total $SiO_2$ -----                                                                                     | about 10    |
| $Na_2O$ -----                                                                                           | about 10.40 |
| Total $SO_3$ (of which 16.4% is titratable $SO_3$ )-----                                                | about 30    |
| Insoluble -----                                                                                         | about 3     |
| Total water (of which about 19 parts can be eliminated only by prolonged heating at 160° to 450°) ----- | about 26.60 |
| Total -----                                                                                             | 100.00      |

In this product the ratio

$$\frac{ZrO_2}{SO_3} \text{ is about } \frac{1}{1.28}$$

which corresponds to a basicity of 36° on the Schorlemer scale.

The complex compound of zirconium dissolves slowly in water, about 3 hours being necessary to obtain complete dissolution.

#### EXAMPLE B

245 kgs. of the ground dry sodium silico-zirconate frit, are rapidly introduced into 146 kgs. of HCl as a 20° Bé. acid solution (s. g. 1.16, 33% HCl) which contains 372 grams HCl per liter. Thus, there are used a total of 390 liters of this acid of 1.16 s. g. equivalent to 452 kgs.

After agitating the mixture for some minutes, the reaction commences. When the temperature of the mixture has risen to about 107° C. the same is allowed to cool giving thereby a yellowish easily pulverizable mass which is almost dry.

After being cooled, there remains about 610 kgs. of a product having approximately the following analysis:

|                                                                                                          | Percent    |
|----------------------------------------------------------------------------------------------------------|------------|
| $ZrO_2$ -----                                                                                            | about 19   |
| NaCl -----                                                                                               | about 18.8 |
| Active Cl combined with $ZrO_2$ and titratable -----                                                     | about 11.3 |
| $H_2O$ -----                                                                                             | about 40.  |
| Insoluble -----                                                                                          | about 3    |
| $SiO_2$ (in form of silica gel, voluminous, having absorbing capacity and substantially insoluble) ----- | about 9.8  |

Another novel feature of this invention comprises the tanning of skins or hides in a bath containing the zirconium tanning agent obtained according to the above procedure. This zirconium tanning product constitutes a water soluble complex salt of zirconium dispersed or absorbed in a voluminous silica gel, the proportion of silica per mole of  $ZrO_2$  being 0.1 to 2 moles and preferably 0.2-1.3 moles. The soluble

zirconium salt dissolves slowly in the tanning bath, during a period of about  $\frac{1}{2}$  to 4 hours, due to the presence of the silica gel which coats the grains of soluble zirconium salt and remains suspended in the bath. The pH of the bath is between 0.5-2, preferably between 0.5-1.9 in order to maintain the zirconium salt in solution and effect tanning of the skins. At a higher pH, the zirconium salt gives colloids deteriorating the tanning properties of the bath. The desired tanning is obtained with a concentration of 10-70 gms. and preferably 25 gms. of zirconium salt, calculated as  $ZrO_2$ , per liter of tanning solution. The silica is in the form of a silica gel and exerts only a physical or physico-chemical effect on the tanning bath, wherein the soluble complex zirconium salt is the effective tanning agent.

20 The soluble  $ZrO_2$  content of the tanning bath, the  $SiO_2:ZrO_2$  molecular ratio and the pH of the bath should be the same as defined above.

25 The following examples are additionally illustrative of the process of tanning with the novel tanning agents of the instant invention, and are not to be construed as limiting the scope thereof.

#### Example 1

For tanning 1 kg. of pickled sheepskins (pH about 2) the following bath can be used:

|                                                                                                                                                                                           |           |
|-------------------------------------------------------------------------------------------------------------------------------------------------------------------------------------------|-----------|
| Water -----                                                                                                                                                                               | 2,000 cc. |
| NaCl -----                                                                                                                                                                                | 160 gms.  |
| Product of the sulfuric acid attack upon sodium silico-zirconate frit, as per Example A, at 20% $ZrO_2$ and at a Schorlemer basicity of about 40° (i. e. about 50 gms. of $ZrO_2$ ) ----- | 250 gms.  |

30 After slowly dissolving the tanning product, the bath contains about 25 gms. of silica ( $SiO_2$ ) in the form of an insoluble voluminous silica gel, having absorptive capacities. The grains of said gel are such that they cannot substantially penetrate into the skin.

35 The skins are agitated in the bath for 3 hours; then permitted to stand overnight or in the tanning solution or on a support. Then the skins are neutralized to about a pH of 4.5 by slowly adding to the bath sodium bicarbonate, borax or any other neutralizing agent.

40 The skins are permitted to stand 24 hours in the vat or on the support and washed to remove soluble salts and adhering silica gel. The skins are then finished in any known manner.

45 The leathers obtained are very white, very full, have an excellent feel to the touch and a very beautiful hair-side.

#### Example 2

50 For 1 kg. of pickled sheepskins (pH about 2) the tanning bath may be as follows:

|                                            |           |
|--------------------------------------------|-----------|
| Water -----                                | 2 liters  |
| Sodium sulphate crystallized -----         | 280 grams |
| Product of Example B (made with HCl) ----- | 260 grams |

55 (of which about 50 grams  $ZrO_2$  is dissolved in the bath). The bath contains about 24 grams of insoluble silica gel ( $SiO_2$ ), having absorptive properties.

60 The skins are agitated in the bath for 3 hours, and neutralized by adding borax to obtain a pH of about 2.8 or 3. After standing for several hours,  $NaHCO_3$  is added to raise the pH to 4-4.5. The skins remain in the bath overnight and are

then washed to remove silica, and finished in the usual way.

The leather is a little less white than the product of Example 1. It is well tanned, very full and has a very pleasing appearance and a good bloom.

Skins and hides other than pickled sheepskins can be tanned in accordance with the instant invention such as horse, calf, beef, cattle, etc. The type of hide used will determine the length of time of the skins' sojourn in the tanning bath and the quantity of  $ZrO_2$  fixed in the skin which is usually between 12 and 24% of the dry leather.

The invention has been described with respect to certain specified examples and preferred methods, but it will be appreciated by those skilled in the art that suitable variations and modifications of the invention may be made without departing from the principles and real spirit of the invention.

What is desired to be secured by Letters Patent is:

1. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter.

2. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium salts in the proportion of 0.1-2 moles  $SiO_2$  per each mole of  $ZrO_2$ , said bath containing 25 gms. zirconium salt calculated as  $ZrO_2$  per liter.

3. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter, the pH of said tanning bath being less than 2.

4. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter, the pH of said tanning bath being between 0.5-2.

5. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter, said water soluble com-

plex of inorganic sodium zirconium salts being partly dissolved in the water of said bath and partly still distributed through and embedded in said silica gel.

6. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium sulfate salts represented by the ratio:

$$\frac{ZrO_2}{SO_3} = \frac{1}{0.8 \text{ to } 2.2}$$

said bath containing 10-70 gms. zirconium salt calculated as  $ZrO_2$  per liter.

7. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium sulfate salts represented by the ratio:

$$\frac{ZrO_2}{SO_3} = \frac{1}{0.8 \text{ to } 2.2}$$

said bath containing 10-70 gms. zirconium salt calculated as  $ZrO_2$  per liter, the pH of said tanning bath being between 0.5-2.

8. A tanning bath essentially consisting of an aqueous suspension of discrete silica gel particles being substantially water insoluble and having a greater than colloidal size, said silica gel particles having distributed therethrough and embedded therein a water soluble complex of inorganic sodium zirconium chloride salts represented by the ratio:

$$\frac{ZrO_2}{HCl} = \frac{1}{1.6 \text{ to } 4}$$

said bath containing 10-70 gms. zirconium salt calculated as  $ZrO_2$  per liter.

9. A process of tanning skins and hides to obtain a superior quality leather, comprising the steps of treating pickled skins with an aqueous tanning bath essentially consisting of an aqueous suspension of discrete silica gel particles being substantially water insoluble, having a greater than colloidal size and being larger than the pores of the pickled skins, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter, so that said silica gel slowly releases said inorganic sodium zirconium salts into the water in contact with the skins, thereby tanning the same; allowing the skins to remain in contact with said tanning bath until the skin is thoroughly tanned; and recovering a superior quality leather.

10. A process of tanning skins and hides to obtain a superior quality leather, comprising the steps of treating pickled skins with an aqueous tanning bath having a pH of less than 2 and essentially consisting of an aqueous suspension of discrete silica gel particles being substantially water insoluble, having a greater than colloidal size and being larger than the pores of the pickled skins, said silica gel particles having distributed therethrough and embedded therein a water soluble complex of inorganic sodium zirconium salts in the proportion of 0.1-2 moles  $SiO_2$  per each

mole of  $ZrO_2$ , said bath containing 10-70 gms. zirconium salt calculated as  $ZrO_2$  per liter, so that said silica gel slowly releases said inorganic sodium zirconium salts into the water in contact with the skins, thereby tanning the same; allowing the skins to remain in contact with said tanning bath until the skin is thoroughly tanned; and recovering a superior quality leather.

11. A process of tanning skins and hides to obtain a superior quality leather, comprising the steps of treating pickled skins with an aqueous tanning bath having a pH between 0.5-1.9 and essentially consisting of an aqueous suspension of discrete silica gel particles being substantially water insoluble, having a greater than colloidal size and being larger than the pores of the pickled skins, said silica gel particles having distributed therethrough and embedded therein a water soluble complex of inorganic sodium zirconium salts in the proportion of 0.1-2 moles  $SiO_2$  per each mole of  $ZrO_2$ , said bath containing 10-70 gms. zirconium salt calculated as  $ZrO_2$  per liter, so that said silica gel slowly releases said inorganic sodium zirconium salts into the water in contact with the skins, thereby tanning the same; allowing the skins to remain in contact with said tanning bath until the skin is thoroughly tanned; and recovering a superior quality leather containing 12-24%  $ZrO_2$ .

12. A product useful for tanning, comprising a water-soluble complex of inorganic sodium zirconium salts, said water-soluble complex being distributed through and embedded in discrete silica gel particles being substantially water-insoluble and having in water a particle size greater than colloidal size, the amount of silica gel per mole of  $ZrO_2$  being 0.2-2.0 moles.

13. A product useful for tanning, comprising a water-soluble complex of inorganic sodium zirconium salts, said water-soluble complex being distributed through and embedded in discrete silica gel particles being substantially water-insoluble and having in water a particle size greater than colloidal size, the amount of silica gel per mole of  $ZrO_2$  being 0.2-1.3 moles.

14. A product useful for tanning, comprising a water-soluble complex of inorganic sodium zirconium sulfate salts, said water-soluble complex being distributed through and embedded in discrete silica gel particles being substantially water insoluble and having in water a particle size greater than colloidal size, the amount of silica gel per mole of  $ZrO_2$  being 0.2-2.0 moles.

15. A product useful for tanning, comprising a water-soluble complex of inorganic sodium zirconium chloride salts, said water-soluble complex being distributed through and embedded in discrete silica gel particles being substantially water-insoluble and having in water a particle size greater than colloidal size, the amount of silica gel per mole of  $ZrO_2$  being 0.2-2.0 moles.

16. A product useful for tanning, comprising a water-soluble complex of inorganic sodium zirconium sulfate salts and having a molecular composition represented by the following ratio:

$$\frac{ZrO_2}{SO_3} = \frac{1}{0.8-2.2}$$

said complex salt being distributed through and embedded in discrete silica gel particles being substantially water-insoluble and having in water a particle size greater than colloidal size, the amount of silica gel per mole of  $ZrO_2$  being 0.2-2.0 moles.

17. A product useful for tanning, comprising

75

a water-soluble complex of inorganic sodium zirconium sulfate salts and having a molecular composition represented by the following ratio:

$$\frac{ZrO_2}{SO_3} = \frac{1}{1.2-1.8}$$

said complex salt being distributed through and embedded in discrete silica gel particles being substantially water-insoluble and having in water a particle size greater than colloidal size, the amount of silica gel per mole of  $ZrO_2$  being 0.2-2.0 moles.

18. A product useful for tanning, comprising a water-soluble complex of inorganic sodium zirconium chloride salts and having a molecular composition represented by the following ratio:

$$\frac{ZrO_2}{HCl} = \frac{1}{1.6-4}$$

20 said complex salt being distributed through and embedded in discrete silica gel particles being substantially water-insoluble and having in water a particle size greater than colloidal size, the amount of silica gel per mole of  $ZrO_2$  being 0.2-2.0 moles.

19. A product useful for tanning, comprising a water-soluble complex of inorganic sodium zirconium chloride salts and having a molecular composition represented by the following ratio:

$$\frac{ZrO_2}{HCl} = \frac{1}{1.8-2.6}$$

said complex salt being distributed through and embedded in discrete silica gel particles being substantially water-insoluble and having in water a particle size greater than colloidal size, the amount of silica gel per mole of  $ZrO_2$  being 0.2-2.0 moles.

20. A process of obtaining a water-soluble complex of inorganic sodium zirconium salts distributed through and embedded in discrete silica gel particles being substantially water-insoluble and having in water a particle size greater than colloidal size, which comprises treating sodium silico-zirconate with sufficient concentrated mineral acid to convert all of the sodium and zirconium into their water-soluble salts of the mineral acid while raising the temperature of the reaction mass to above 105° C., and recovering a substantially dry, pulverulent solid product composed of a water-soluble complex of inorganic sodium zirconium salts distributed through and embedded in discrete silica gel particles.

45 21. A process of obtaining a water-soluble complex of inorganic sodium zirconium salts distributed through and embedded in discrete silica gel particles being substantially water-insoluble and having in water a particle size greater than colloidal size, which comprises calcining a silica-containing zirconium ore with sodium carbonate to produce sodium silico-zirconate, treating said sodium silico-zirconate with sufficient concentrated mineral acid to convert all of the sodium and zirconium into their water-soluble salts of the mineral acid while raising the temperature of the reaction mass to above 105° C., and recovering a substantially dry, pulverulent solid product composed of a water-soluble complex of inorganic sodium zirconium salts distributed through and embedded in discrete silica gel particles.

60 22. A process of obtaining a water-soluble complex of inorganic sodium zirconium salts distributed through and embedded in discrete silica gel particles being substantially water-insoluble and having in water a particle size greater than colloidal size, which comprises calcining a silica-containing zirconium ore with sodium carbonate to produce sodium silico-zirconate, treating said sodium silico-zirconate with sufficient concentrated mineral acid to convert all of the sodium and zirconium into their water-soluble salts of the mineral acid while raising the temperature of the reaction mass to above 105° C., and recovering a substantially dry, pulverulent solid product composed of a water-soluble complex of inorganic sodium zirconium salts distributed through and embedded in discrete silica gel particles.

65 23. A process of obtaining a water-soluble complex of inorganic sodium zirconium salts distributed through and embedded in discrete silica gel particles being substantially water-insoluble and having in water a particle size greater than colloidal size, which comprises calcining a silica-containing zirconium ore with sodium carbonate to produce sodium silico-zirconate, treating said sodium silico-zirconate with sufficient concentrated mineral acid to convert all of the sodium and zirconium into their water-soluble salts of the mineral acid while raising the temperature of the reaction mass to above 105° C., and recovering a substantially dry, pulverulent solid product composed of a water-soluble complex of inorganic sodium zirconium salts distributed through and embedded in discrete silica gel particles.

70 24. A process of obtaining a water-soluble complex of inorganic sodium zirconium salts distributed through and embedded in discrete silica gel particles being substantially water-insoluble and having in water a particle size greater than colloidal size, which comprises calcining a silica-containing zirconium ore with sodium carbonate to produce sodium silico-zirconate, treating said sodium silico-zirconate with sufficient concentrated mineral acid to convert all of the sodium and zirconium into their water-soluble salts of the mineral acid while raising the temperature of the reaction mass to above 105° C., and recovering a substantially dry, pulverulent solid product composed of a water-soluble complex of inorganic sodium zirconium salts distributed through and embedded in discrete silica gel particles.

## 11

silica gel particles being substantially water-insoluble and having in water a particle size greater than colloidal size, which comprises treating sodium silico-zirconate with sufficient concentrated sulfuric acid to convert all of the sodium and zirconium into their water-soluble salts of the mineral acid having the molecular composition represented by the ratio:

$$\frac{\text{ZrO}_2}{\text{SO}_3} = \frac{1}{0.8-2.2}$$

while raising the temperature of the reaction mass to above 105° C., and recovering a substantially dry, pulverulent solid product composed of a water soluble complex of inorganic sodium zirconium sulfate salts distributed through and embedded in discrete silica gel particles.

23. A process of obtaining a water-soluble complex of inorganic sodium zirconium salts distributed through and embedded in discrete silica gel particles being substantially water-insoluble and having in water a particle size greater than colloidal size, which comprises treating sodium silico-zirconate with sufficient concentrated hydrochloric acid to convert all of the sodium and zirconium into their water-soluble salts of the mineral acid having the molecular composition represented by the ratio:

$$\frac{\text{ZrO}_2}{\text{HCl}} = \frac{1}{0.6-4}$$

while raising the temperature of the reaction mass to above 105° C., and recovering a substantially dry, pulverulent solid product composed of a water soluble complex of inorganic sodium zirconium chloride salts distributed through and embedded in discrete silica gel particles.

24. A process of obtaining a water-soluble complex of inorganic sodium zirconium salts distributed through and embedded in discrete silica gel particles being substantially water-insoluble and having in water a particle size greater than colloidal size, which comprises treating sodium silico-zirconate with sufficient concentrated sulfuric acid having a concentration between 35°-60° Bé. to convert all of the sodium and zirconium into their water-soluble salts of the mineral acid having the molecular composition represented by the ratio:

$$\frac{\text{ZrO}_2}{\text{SO}_3} = \frac{1}{0.8-2.2}$$

while raising the temperature of the reaction mass to above 105° C., and recovering a substantially

## 12

dry, pulverulent solid product composed of a water-soluble complex of inorganic sodium zirconium sulfate salts distributed through and embedded in discrete silica gel particles.

- 5 25. A process of obtaining a water-soluble complex of inorganic sodium zirconium salts distributed through and embedded in discrete silica gel particles being substantially water-insoluble and having in water a particle size greater than colloidal size, which comprises treating sodium silico-zirconate with sufficient concentrated hydrochloric acid having a concentration between 13°-22° Bé. to convert all of the sodium and zirconium into their water-soluble salts of the mineral acid having the molecular composition represented by the ratio:

$$\frac{\text{ZrO}_2}{\text{HCl}} = \frac{1}{0.6-4}$$

- 10 20 while raising the temperature of the reaction mass to above 105° C., and recovering a substantially dry, pulverulent solid product composed of a water soluble complex of inorganic sodium zirconium chloride salts distributed through and embedded in discrete silica gel particles.

- 15 25 26. A process of obtaining a water-soluble complex of inorganic sodium zirconium salts distributed through and embedded in discrete silica gel particles being substantially water-insoluble and having in water a particle size greater than colloidal size, which comprises treating sodium silico-zirconate with sufficient concentrated concentrated mineral acid to convert all of the sodium and zirconium into their water-soluble salts of the mineral acid while raising the temperature of the reaction mass to about 110-120° C., and recovering a substantially dry, pulverulent solid product composed of a water soluble complex of inorganic sodium zirconium salts distributed through and embedded in discrete silica gel particles.

## References Cited in the file of this patent

## UNITED STATES PATENTS

| Number    | Name                  | Date           |
|-----------|-----------------------|----------------|
| 2,127,304 | Mauthe et al. -----   | Aug. 16, 1938  |
| 2,395,472 | Fernald -----         | Feb. 26, 1949  |
| 2,477,638 | Milliken et al. ----- | Aug. 2, 1949   |
| 2,481,493 | Blue -----            | Sept. 13, 1949 |

## FOREIGN PATENTS

| Number  | Country      | Date          |
|---------|--------------|---------------|
| 917,317 | France ----- | Sept. 6, 1946 |